

## 1

3,575,736

**METHOD OF ROLLING TITANIUM ALLOYS**  
John M. Fitzpatrick, Los Altos, and Aloysius T. Davinroy,  
Redwood City, Calif., assignors to the United States  
of America as represented by the Secretary of the Air  
Force  
No Drawing. Filed Nov. 25, 1968, Ser. No. 778,760  
Int. Cl. B21b 1/00, 3/00; B21d 31/00; C21d 1/00  
U.S. Cl. 148—11.5 3 Claims

### ABSTRACT OF THE DISCLOSURE

A method for enhancing the strength to density ratio of alpha-beta type titanium alloys. The increased strength demonstrated by the alloys of this invention is achieved by favorably altering the crystallographic texture of the alloy. The alloy to be textured is hot rolled in at least three different orientations at a temperature within a range of from about 700° to 1500° F. This results in a reduction in the cross-sectional area of the alloy by about 60 to 90%.

### BACKGROUND OF THE INVENTION

This invention relates to a method for hot rolling titanium-base alloys. More particularly, this invention concerns itself with achieving favorable crystallographic texture in titanium-base alloys of the alpha-beta type by subjecting the alloy material to a multi-directional rolling process.

The formulation and fabrication of alloy materials characterized by high strength-to-density ratios has become a problem of paramount importance with the recent advances made in rocket technology. The need for such materials is obvious if further technical advances are to be made. Attempts to fully utilize the inherent potential of titanium alloys to achieve strength-to-density ratios comparable to ratios of fiberglass composites for rocket motor applications has not been successful. It is well known that deformation processing in a combination with heat hardening significantly improves the strength of metal alloys. Amongst titanium alloy the crystallographic texture which is most desirable for providing strength is one in which the basal planes of the hexagonal-alpha-phase lattice are preferentially parallel to the plane of the sheet. This texture provides strength under biaxial stress conditions greater than those in a crystallographically isotropic metal of the same composition. The all alpha alloys of titanium display this classical basal plane texturing after unidirectional rolling but these alloys do not have the potential of being heat treated in order to provide increased strength.

The alpha-beta type titanium alloys are generally rolled in one direction at temperatures of about 1700° F. with resultant textures giving rise to a less-than-isotropic biaxial strength. Although these alloys have not been considered ideally suited for texture hardening, some strength improvement can be achieved through heat hardening. The ability to properly texture harden and significantly improve the strength of alpha-beta titanium alloys is of extreme importance if the maximum utilization of titanium metal is to be realized for rocket motor applications. Previous

## 2

methods of texture hardening by straight rolling, as above, and shear spinning have so far not shown any significant increase in the textured properties of these alloys.

With the present invention, however, it has been found that a heat-treatable, texture-hardened titanium alloy suitable for use in rocket motor cases can be fabricated by subjecting a sheet of the alloy to a multi-directional rolling process preferably at temperatures not to exceed about 1300° F. The alloy work piece is rolled in a direction parallel with respect to the rolling direction. After each successive rolling pass, the work piece is rotated 45° and then reheated. This provides a multi-directional rolling process in which the work piece is rolled in three orientations with respect to the rolling direction: parallel to the rolling direction, transverse to the rolling direction, and at an angle of 45° or diagonal to the rolling direction.

The texture hardening multidirectional rolling process of this invention provides a means for utilizing the full potential of alpha-beta type titanium alloys by favorably altering the crystallographic texture of the alloy. The resultant alloy possesses higher strength under biaxial stress conditions and consequently enable the fabrication of lighter weight structures.

### SUMMARY OF THE INVENTION

In accordance with this invention, texture hardening of alpha-beta type titanium alloys can be accomplished by multi-directional rolling process in which alloy metal sheets are hot rolled in three different orientations at temperatures ranging from about 700° F to 1500° F. The sheets are subjected to successive rolling operations, each of which is alternately oriented along three different directions with respect to the rolling direction: parallel to the rolling direction, transverse to the rolling direction, and at a 45° angle or diagonal to the rolling direction.

Texture hardening in accordance with the process of this invention results in a significant improvement in the strength to weight ratios of alpha-beta titanium alloys as compared to the results achieved by previously known hardening processes. After multi-directional rolling, the alloys display the favorable basal plane texturing in which the basal planes of the hexagonal-alpha-phase lattice are preferentially oriented parallel to the plane of the sheet. This results in the fabrication of a high strength alpha-beta type titanium alloy.

Accordingly, the primary object of this invention is to provide a method for favorably texturing alpha-beta titanium alloys by preferentially orienting the basal plane of the alloy's crystal lattice parallel to the plane of the sheet.

Another object of this invention is to provide a method for fully utilizing the inherent characteristics of titanium alloys to achieve high strength-to-density ratios.

Still another object of this invention is to provide a method for inducing high strength in alpha-beta type titanium alloys through a combination of processing parameters which includes heat treating and deformation-processing.

The above and still further objects and advantages of this invention will become apparent upon consideration of the following detailed description thereof;

**3**  
**DESCRIPTION OF THE PREFERRED**  
**EMBODIMENT**

The present invention is predicated on the discovery that the crystallographic texture of alpha-beta titanium alloys can be favorably altered to produce a classical basal plane texture in order to provide an alpha-beta type titanium alloy having a high strength to density ratio. The favorable alteration is achieved by subjecting an alloy work piece to a series of hot rolling steps oriented in three different directions to reduce its cross-sectional area. The cross-sectional area is ultimately reduced by about 60 to 90 percent and the rolling steps are conducted at temperatures of from about 700 to 1500° F. Preferably the work piece is rolled at a temperature of about 1300° F. and reduced in cross-sectional area by about 90 percent.

Specific examples of alpha-beta type titanium alloys subjected to the rolling process of this invention were of two compositions, Ti-6Al-4V and Ti-7Al-2.5Mo. The Ti-6Al-4V alloy was obtained in the form of  $\frac{3}{4}$  in.-thick strip, 6 in. wide. It had been a ring-rolled forging with a wall thickness of approximately  $1\frac{1}{2}$  in. The ring was cut open, straightened on a forge press at 1750° F., and then rolled from a furnace temperature of 1750° F. to  $\frac{3}{4}$  in. thick. This strip was conditioned to remove oxide and surface irregularities by machining  $\frac{1}{16}$  in. from both surfaces. The resulting plate,  $\frac{5}{8}$  in. thick, was used for processing in accordance with this invention. A second form of a Ti-6Al-4V alloy used in the rolling process was  $1\frac{1}{2}$  in.-thick plate.

The Ti-7Al-2.5Mo alloy was obtained in the form of 2-in. thick plates. This material was converted to thicknesses that could be used on a two-high Fenn rolling mill. Conversion was performed in two ways by a vendor forge shop. The first way was to roll slabs from 2 in. thick to approximately 1 in. thick at a furnace temperature of 1750° F. The second way was to hammer-forged some of the 2-in. thick material to approximately 1 in. thick, also at a furnace temperature of 1750° F. The rolled material was further reduced by rolling on the Fenn mill to  $\frac{5}{8}$ -in. thickness at a furnace temperature of 1750° F. Both the rolled and forged materials were used in preparing multi-directional rolled sheet for test evaluation.

The starting size of the work piece multi-directional rolling was a regular octagon,  $4\frac{1}{2}$  in. across the parallel edges. These starting blanks were prepared from the thick plates ( $1\frac{1}{2}$ -in. thick Ti-6Al-4V and 1-in. thick Ti-7Al-2.5Mo) by cutting the required shape on an abrasive cut-off wheel. Typical rolling schedules are illustrated in Tables I and II for Ti-6Al-4V and Ti-7Al-2.5Mo respectively. On each successive rolling pass, the octagon was rotated 45° and reheated after every pass.

When the size of the work piece reached an effective diameter of 9 in., the octagonal plate was cut into two equal sections from each of which was prepared another regular octagon measuring approximately  $4\frac{1}{2}$  in. across. These pieces were then multi-directionally rolled in the same manner as before to a final thickness of approximately  $\frac{1}{8}$  in. A production summary of multi-directional rolling is given in Table III.

**TABLE I**  
**[Multi-directional rolling schedule for Ti-6Al-4V; Preheat Temperature 1,300° F.]**

| Pass No.                                         | Material thickness | Per cent/ pass | Exit temp. (° F.) | Remarks |
|--------------------------------------------------|--------------------|----------------|-------------------|---------|
| 1.500 ----- Preheat block for 1 hr. at 1,300° F. |                    |                |                   |         |
| 1.                                               | 1.469              | 2.0            | 1,040             |         |
| 2.                                               | 1.416              | 3.7            | -----             |         |
| 3.                                               | 1.372              | 3.1            | -----             |         |
| 4.                                               | 1.322              | 3.6            | -----             |         |
| 5.                                               | 1.223              | 7.0            | 1,050             |         |
| 6.                                               | 1.171              | 4.3            | 1,020             |         |
| 7.                                               | 1.120              | 4.4            | 1,020             |         |
| 8.                                               | 1.071              | 4.4            | 1,040             |         |
| 9.                                               | 1.020              | 4.8            | 1,060             |         |
| 10.                                              | 0.965              | 5.4            | -----             |         |

**4**  
**TABLE I.—Continued**

| Pass No. | Material thickness | Per cent/ pass | Exit temp. (° F.) | Remarks                                                                         |
|----------|--------------------|----------------|-------------------|---------------------------------------------------------------------------------|
| 5        | 0.918              | 4.3            | -----             |                                                                                 |
|          | 0.871              | 5.1            | 1,040             |                                                                                 |
|          | 0.820              | 5.9            | -----             |                                                                                 |
|          | 0.769              | 6.2            | 1,020             |                                                                                 |
|          | 0.722              | 6.1            | -----             |                                                                                 |
|          | 0.672              | 6.9            | 1,000             |                                                                                 |
|          | 0.625              | 7.0            | -----             |                                                                                 |
|          | 0.571              | 8.6            | 1,000             |                                                                                 |
|          | 0.532              | 6.8            | -----             |                                                                                 |
|          | 0.508              | 4.5            | 960               |                                                                                 |
|          | 0.470              | 7.4            | 1,000             | Slight dishing of plate occurred on 21st pass and persisted through final pass. |
|          | 0.445              | 5.3            | -----             |                                                                                 |
|          | 0.426              | 4.3            | 980               |                                                                                 |
|          | 0.406              | 4.7            | -----             |                                                                                 |
|          | 0.389              | 4.7            | 1,000             |                                                                                 |
|          | 0.365              | 5.7            | -----             |                                                                                 |
|          | 0.347              | 4.9            | 1,000             |                                                                                 |
|          | 0.331              | 4.6            | -----             |                                                                                 |
|          | 0.316              | 4.5            | 960               |                                                                                 |
|          | 0.297              | 6.0            | 920               |                                                                                 |
|          | 0.281              | 5.4            | 930               |                                                                                 |
|          | 0.268              | 4.6            | 890               |                                                                                 |
|          | 0.253              | 5.6            | 900               |                                                                                 |
|          | 0.239              | 5.5            | 900               |                                                                                 |
|          | 0.228              | 4.6            | 900               |                                                                                 |
|          | 0.218              | 4.4            | 900               |                                                                                 |
|          | 0.206              | 5.5            | 890               |                                                                                 |
|          | 0.200              | 2.3            | 840               |                                                                                 |
|          | 0.187              | 6.5            | 840               |                                                                                 |
|          | 0.175              | 6.4            | 860               |                                                                                 |
|          | 0.168              | 4.0            | 860               |                                                                                 |
|          | 0.156              | 7.1            | 840               |                                                                                 |
|          | 0.139              | 8.5            | 820               |                                                                                 |
|          | 0.136              | 2.2            | 800               |                                                                                 |
|          | 0.130              | 4.3            | 780               |                                                                                 |
|          | 0.127              | 2.3            | -----             |                                                                                 |

35

40

**TABLE II**  
**[Multi-directional rolling schedule for Ti-7Al-2.5Mo; preheat temperature 1,450° F.]**

| Pass No. | Material thickness | Per cent/ pass | Exit temp. (° F.) | Remarks                                                                         |
|----------|--------------------|----------------|-------------------|---------------------------------------------------------------------------------|
| 45       | 1.000              | -----          | -----             | Preheat block at 1,450° F. for 1 hr.                                            |
|          | 0.926              | 5.6            | 1,100             |                                                                                 |
|          | 0.871              | 5.9            | 1,100             |                                                                                 |
|          | 0.818              | 6.1            | 1,130             |                                                                                 |
|          | 0.768              | 6.1            | 1,100             |                                                                                 |
|          | 0.722              | 6.0            | 1,100             |                                                                                 |
|          | 0.679              | 6.0            | -----             |                                                                                 |
|          | 0.637              | 6.2            | 1,100             |                                                                                 |
|          | 0.600              | 5.8            | 1,100             |                                                                                 |
|          | 0.563              | 6.2            | 1,100             |                                                                                 |
|          | 0.530              | 5.9            | -----             |                                                                                 |
|          | 0.498              | 6.0            | 1,080             |                                                                                 |
|          | 0.467              | 6.2            | -----             |                                                                                 |
|          | 0.440              | 5.8            | 1,070             |                                                                                 |
|          | 0.414              | 5.9            | -----             |                                                                                 |
|          | 0.390              | 5.8            | 1,040             |                                                                                 |
|          | 0.367              | 6.0            | 1,040             |                                                                                 |
|          | 0.344              | 6.3            | 1,040             |                                                                                 |
|          | 0.326              | 5.2            | 1,040             |                                                                                 |
|          | 0.307              | 5.8            | 1,040             |                                                                                 |
|          | 0.290              | 5.5            | 980               | Slight dishing of plate occurred on 20th pass and persisted through final pass. |
|          | 0.272              | 6.2            | -----             |                                                                                 |
|          | 0.262              | 3.7            | 1,020             |                                                                                 |
|          | 0.249              | 5.0            | 940               |                                                                                 |
|          | 0.234              | 6.0            | 960               |                                                                                 |
|          | 0.221              | 5.0            | -----             |                                                                                 |
|          | 0.210              | 5.0            | 900               |                                                                                 |
|          | 0.200              | 4.8            | 900               |                                                                                 |
|          | 0.188              | 6.0            | 940               |                                                                                 |
|          | 0.182              | 3.2            | 940               |                                                                                 |
|          | 0.173              | 5.0            | -----             |                                                                                 |
|          | 0.164              | 5.2            | 800               |                                                                                 |
|          | 0.155              | 5.5            | 880               |                                                                                 |
|          | 0.148              | 4.5            | 880               |                                                                                 |
|          | 0.143              | 3.4            | 860               |                                                                                 |
|          | 0.136              | 4.9            | -----             |                                                                                 |
|          | 0.129              | 5.1            | 840               |                                                                                 |
|          | 0.127              | 1.6            | 840               |                                                                                 |
|          | 0.123              | 3.1            | 800               |                                                                                 |
|          | 0.123              | -----          | -----             |                                                                                 |

75

TABLE III  
Ti-6 Al-4V and Ti-7Al-2.5Mo multi-directional roll production summary

| Alloy        | Sheet designation | Material starting thickness (in.) | Pre-heat temp. (° F.) <sup>1</sup> | Total reduction (percent) | Total rolling passes | Remarks                                                                                                                                                      |
|--------------|-------------------|-----------------------------------|------------------------------------|---------------------------|----------------------|--------------------------------------------------------------------------------------------------------------------------------------------------------------|
| Ti-6Al-4V    | 3SRR              | 1.5                               | 1,300                              | 93                        | 47                   | Two plates obtained with a diameter of 8 in.                                                                                                                 |
| Ti-6Al-4V    | 4SRR              | 1.5                               | 1,300                              | 91.5                      | 49                   | Four plates obtained with a diameter of 7½ in.                                                                                                               |
| Ti-6Al-4V    | 8SRR              | 0.624                             | 1,300                              | 80                        | 25                   | Straight rolled at furnace temperature 1,700° F. from 1½ in. thick to 0.625 in. prior to round rolling. Two finished plates obtained with diameter of 8½ in. |
| Ti-6Al-4V    | 10SRR             | 0.624                             | 1,100                              | 80                        | 27                   | Do.                                                                                                                                                          |
| Ti-6Al-4V    | 13SRR             | 0.370                             | 1,300                              | 70                        | 20                   | Straight rolled at furnace temperature 1,700° F. from 1½ in. thick to 0.370 in. prior to round rolling. Two finished plates obtained with diameter of 7½ in. |
| Ti-6Al-4V    | 15SRR             | 0.370                             | 1,100                              | 70                        | 22                   | Do.                                                                                                                                                          |
| Ti-6Al-4V    | 17SRR             | 1.5                               | 1,400                              | 92                        | 43                   | Two plates obtained with a diameter of 7½ in.                                                                                                                |
| Ti-6Al-4V    | 19SRR             | 1.5                               | 1,500                              | 92                        | 40                   | Do.                                                                                                                                                          |
| Ti-7Al-2.5Mo | 12SRR             | 0.620                             | 1,400                              | 80                        | 24                   | One plate obtained with a diameter of 10 in.                                                                                                                 |
| Ti-7Al-2.5Mo | 24SRR             | 1.000                             | 1,450                              | 87                        | 38                   | Do.                                                                                                                                                          |

<sup>1</sup> The preheat temperature is that at which the material was allowed to soak. This soaking was performed in a 40 kw. resistance box furnace for 15 min. prior to each rolling pass. Whenever the material was allowed to air cool, it was preheated for a period of not less than 30 min. prior to the next rolling pass.

No conditioning was necessary for the Ti-6Al-4V alloys other than that described heretofore. The 1½ in. thick plate was received as bright, flat, and locally conditioned material. The hammer-forged Ti-7Al-2.5Mo alloy required milling approximately 1/16 in. from both surfaces to prepare clean, flat surfaces for rolling.

All rolling procedures were done on a Fenn, type 081, two-high rolling mill. The mill had a ground, roll-face width of 9 in. Unidirectional rolling (also termed straight rolling) was conducted on starting plates (sheet-bars) of the Ti-6Al-4V having the following dimensions: 7½ by 8¾ by 1½ in. Unidirectional rolling was carried out with the 7½-in. dimension in the rolling direction. Rolled sheets were edge trimmed by shearing or abrasive wheel cutting to 8-in. widths in order to pass through the Stanat Roller Leveler. The roller-leveler was employed following the final roll pass to achieve necessary flatness in the sheets. In some cases, the work had a tendency to curl on exit from the rolls, particularly at thicknesses between ½ and ¼ in. When this occurred, it was necessary to flatten the pieces on a hydraulic press between platens. Prior to a flattening or roller leveling operation, the work was heated to the same temperature as it would be for a rolling pass. Typical unidirectional rolling schedules are shown in Tables IV and V and were conducted to provide comparative results achieved between unidirectional and multi-directional rolling. All rolling was done at a constant roll speed of 29 ft./min., which was chosen only for convenience in handling the material on exit from the mill. The actual temperature of the metal on exit from the rolls was monitored periodically with a surface-contact pyrometer. The work was reheated to the furnace temperature after each pass. Percentage reduction per pass was determined by a limit imposed by the strength of shear pins in the drive train of the rolling mill. A production summary of straight rolling is given in Table VI.

TABLE IV  
[Unidirectional rolling schedule for Ti-6Al-4V; preheat temperature 1,100° F.]

| Pass No. | Material thickness | Percent/ temp. pass | Exit temp. (° F.) | Remarks                                                                                                                      |
|----------|--------------------|---------------------|-------------------|------------------------------------------------------------------------------------------------------------------------------|
| 1.       | 1.522              | 1.7                 |                   | Preheat block at 1,100° F. for 1 hr.                                                                                         |
| 2.       | 1.496              | 1.7                 |                   |                                                                                                                              |
| 3.       | 1.478              | 1.2                 |                   |                                                                                                                              |
| 4.       | 1.458              | 1.3                 |                   |                                                                                                                              |
| 5.       | 1.441              | 1.2                 |                   |                                                                                                                              |
| 6.       | 1.421              | 1.4                 |                   |                                                                                                                              |
| 7.       | 1.401              | 1.4                 |                   |                                                                                                                              |
| 8.       | 1.381              | 1.0                 |                   |                                                                                                                              |
| 9.       | 1.365              | 1.16                |                   |                                                                                                                              |
| 10.      | 1.343              | 1.6                 | 940               |                                                                                                                              |
| 11.      | 1.324              | 1.55                | 900               |                                                                                                                              |
| 12.      | 1.306              | 1.38                | 900               |                                                                                                                              |
| 13.      | 1.286              | 1.5                 | 900               |                                                                                                                              |
| 14.      | 1.264              | 1.7                 | 900               |                                                                                                                              |
| 15.      | 1.245              | 1.5                 | 900               |                                                                                                                              |
| 16.      | 1.223              | 1.77                | 900               |                                                                                                                              |
| 17.      | 1.202              | 1.7                 |                   |                                                                                                                              |
| 18.      | 1.181              | 1.75                | 940               |                                                                                                                              |
| 19.      | 1.162              | 1.6                 |                   |                                                                                                                              |
| 20.      |                    |                     |                   |                                                                                                                              |
| 21.      |                    |                     |                   |                                                                                                                              |
| 22.      |                    |                     |                   |                                                                                                                              |
| 23.      |                    |                     |                   |                                                                                                                              |
| 24.      |                    |                     |                   |                                                                                                                              |
| 25.      |                    |                     |                   |                                                                                                                              |
| 26.      |                    |                     |                   |                                                                                                                              |
| 27.      |                    |                     |                   |                                                                                                                              |
| 28.      |                    |                     |                   |                                                                                                                              |
| 29.      |                    |                     |                   |                                                                                                                              |
| 30.      |                    |                     |                   |                                                                                                                              |
| 31.      |                    |                     |                   |                                                                                                                              |
| 32.      |                    |                     |                   |                                                                                                                              |
| 33.      |                    |                     |                   |                                                                                                                              |
| 34.      |                    |                     |                   |                                                                                                                              |
| 35.      |                    |                     |                   |                                                                                                                              |
| 36.      |                    |                     |                   |                                                                                                                              |
| 37.      |                    |                     |                   |                                                                                                                              |
| 38.      |                    |                     |                   |                                                                                                                              |
| 39.      |                    |                     |                   |                                                                                                                              |
| 40.      |                    |                     |                   | Press-straighten plate after 40th pass.                                                                                      |
| 41.      |                    |                     |                   | Press-straighten plate after 42nd pass.                                                                                      |
| 42.      |                    |                     |                   | Press-straighten plate after 44th pass.                                                                                      |
| 43.      |                    |                     |                   | Press-straighten plate after 46th pass.                                                                                      |
| 44.      |                    |                     |                   | Press-straighten plate after 48th pass.                                                                                      |
| 45.      |                    |                     |                   | Press-straighten plate after 50th pass.                                                                                      |
| 46.      |                    |                     |                   | Press-straighten plate after 52nd pass. Plate now measures 26½ in. long and will be cut in half for continuation of rolling. |
| 47.      |                    |                     |                   |                                                                                                                              |
| 48.      |                    |                     |                   |                                                                                                                              |
| 49.      |                    |                     |                   |                                                                                                                              |
| 50.      |                    |                     |                   |                                                                                                                              |
| 51.      |                    |                     |                   |                                                                                                                              |
| 52.      |                    |                     |                   |                                                                                                                              |
| 53.      |                    |                     |                   |                                                                                                                              |
| 54.      |                    |                     |                   |                                                                                                                              |
| 55.      |                    |                     |                   |                                                                                                                              |
| 56.      |                    |                     |                   |                                                                                                                              |
| 57.      |                    |                     |                   |                                                                                                                              |
| 58.      |                    |                     |                   |                                                                                                                              |
| 59.      |                    |                     |                   |                                                                                                                              |
| 60.      |                    |                     |                   |                                                                                                                              |
| 61.      |                    |                     |                   |                                                                                                                              |
| 62.      |                    |                     |                   |                                                                                                                              |
| 63.      |                    |                     |                   |                                                                                                                              |
| 64.      |                    |                     |                   |                                                                                                                              |
| 65.      |                    |                     |                   |                                                                                                                              |
| 66.      |                    |                     |                   |                                                                                                                              |
| 67.      |                    |                     |                   |                                                                                                                              |
| 68.      |                    |                     |                   |                                                                                                                              |
| 69.      |                    |                     |                   |                                                                                                                              |
| 70.      |                    |                     |                   |                                                                                                                              |
| 71.      |                    |                     |                   |                                                                                                                              |
| 72.      |                    |                     |                   |                                                                                                                              |
| 73.      |                    |                     |                   |                                                                                                                              |
| 74.      |                    |                     |                   |                                                                                                                              |
| 75.      |                    |                     |                   |                                                                                                                              |
| 76.      |                    |                     |                   |                                                                                                                              |
| 77.      |                    |                     |                   |                                                                                                                              |
| 78.      |                    |                     |                   |                                                                                                                              |
| 79.      |                    |                     |                   |                                                                                                                              |
| 80.      |                    |                     |                   |                                                                                                                              |
| 81.      |                    |                     |                   |                                                                                                                              |
| 82.      |                    |                     |                   |                                                                                                                              |
| 83.      |                    |                     |                   |                                                                                                                              |
| 84.      |                    |                     |                   | Air-cool sheet after final pass.                                                                                             |

TABLE V

[Unidirectional rolling schedule for Ti-6Al-4V; preheat temperature 1300° F.]

| Pass. No. | Material thickness | Per cent/ pass | Exit temp. (° F.) | Remarks                                 |
|-----------|--------------------|----------------|-------------------|-----------------------------------------|
| 1.        | 1.500              |                |                   | Preheat block for 1 hr. at 1300° F.     |
| 1.        | 1.448              |                | 1,050             |                                         |
| 2.        | 1.426              | 2.2            | 1,050             |                                         |
| 3.        | 1.380              | 3.2            |                   |                                         |
| 4.        | 1.332              | 3.48           | 1,050             |                                         |
| 5.        | 1.280              | 3.9            |                   |                                         |
| 6.        | 1.230              | 3.9            | 1,050             |                                         |
| 7.        | 1.180              | 4.1            |                   |                                         |
| 8.        | 1.127              | 4.5            | 1,050             |                                         |
| 9.        | 1.079              | 4.25           |                   |                                         |
| 10.       | 1.030              | 4.5            | 1,050             |                                         |
| 11.       | 0.977              | 5.1            |                   |                                         |
| 12.       | 0.926              | 5.2            | 1,050             |                                         |
| 13.       | 0.877              | 5.3            |                   |                                         |
| 14.       | 0.828              | 5.6            |                   |                                         |
| 15.       | 0.775              | 6.4            |                   |                                         |
| 16.       | 0.725              | 6.5            |                   |                                         |
| 17.       | 0.676              | 6.75           |                   |                                         |
| 18.       | 0.629              | 6.9            |                   |                                         |
| 19.       | 0.594              | 6.5            |                   | Press-straighten plate after 19th pass. |
| 20.       | 0.559              | 5.9            |                   |                                         |
| 21.       | 0.522              | 6.6            |                   |                                         |
| 22.       | 0.494              | 5.4            |                   | Press-straighten plate after 22nd pass. |
| 23.       | 0.464              | 6.1            |                   |                                         |
| 24.       | 0.438              | 5.6            |                   |                                         |
| 25.       | 0.409              | 6.6            |                   | Press-straighten plate after 25th pass. |
| 26.       | 0.384              | 6.1            |                   |                                         |
| 27.       | 0.362              | 5.7            |                   | Press-straighten plate after 27th pass. |
| 28.       | 0.342              | 5.5            |                   |                                         |
| 29.       | 0.320              | 6.4            |                   |                                         |
| 30.       | 0.308              | 3.8            |                   |                                         |
| 31.       | 0.302              | 4.7            | 980               | Press-straighten plate after 31st pass. |
| 32.       | 0.284              | 6.0            | 980               |                                         |
| 33.       | 0.270              | 4.9            | 960               | Press-straighten plate after 33rd pass. |
| 34.       | 0.252              | 6.7            |                   | Press-straighten plate after 34th pass. |
| 35.       | 0.235              | 6.7            |                   |                                         |
| 36.       | 0.223              | 5.1            |                   |                                         |
| 37.       | 0.209              | 6.3            | 900               |                                         |
| 38.       | 0.195              | 6.7            |                   |                                         |
| 39.       | 0.183              | 6.2            | 840               |                                         |
| 40.       | 0.171              | 6.5            | 880               |                                         |
| 41.       | 0.159              | 7.0            |                   |                                         |
| 42.       | 0.152              | 0.4            |                   | Air-cool sheet after final pass.        |

Uniaxial tension test data for the  $\frac{5}{8}$ -in.-thick Ti-6Al-4V alloy material are presented in Table VII. Here, the uniaxial test data for the as-received plate, as well as data on straight-rolled and multi-directional rolled plates are shown. On the basis of the R values, this material appears to be capable of developing substantial textures during rolling to a total reduction of about 80%.

Uniaxial tension test data for the Ti-7Al-2.5Mo alloy in the hammer-forged condition are presented in Table VIII. In this case, we find that R is slightly greater than 1, and that substantial R values are achieved by multi-directional rolling to total reductions of less than 90%.

TABLE VII

15 Uniaxial tension data on preliminary material (Ti-6Al-4V) in indicated condition

|     | Longitudinal                                                   |
|-----|----------------------------------------------------------------|
| 20. | Yield strength at 0.2% (k.s.i.) ----- 102.2                    |
|     | Engineering tensile strength (k.s.i.) ----- 142.0              |
|     | Young's modulus (p.s.i. $\times 10^{-6}$ ) ----- 13.45         |
|     | Plastic strain at maximum load (percent) ----- 4.6             |
|     | Total elongation (2-in. gage) (percent) ----- 13.3             |
| 25. | Elastic Poisson's ratio ----- 0.349                            |
|     | R at 0.2% long. plastic strain ----- 0.8                       |
|     | Calculated 1:2 biaxial YS (k.s.i.) ----- 113.6                 |
|     | As-received.                                                   |
| 30. | Yield strength at 0.2% (k.s.i.) ----- 150.3                    |
|     | Engineering tensile strength (k.s.i.) ----- 168.7              |
|     | Young's modulus (p.s.i. $\times 10^{-6}$ ) ----- 14.8          |
|     | Plastic strain at maximum load (percent) ----- 2.6             |
|     | Total elongation (2-in. gage) (percent) ----- 4.0              |
| 35. | Elastic Poisson's ratio ----- 0.393                            |
|     | R at 0.2% long. plastic strain ----- 3.07                      |
|     | Calculated 1:2 biaxial YS (k.s.i.) ----- 214.0                 |
| 40. | Straight rolled ~ 80% furnace temperature 1100° F., as-rolled. |

TABLE VI

[Ti-6Al-4V unidirectional sheet production summary]

| Sheet designation | Material starting thickness (in.) | Pre-heat temp. (° F.) <sup>1</sup> | Total reduction (percent) | Total rolling passes | Remarks                                                                                                                                  |
|-------------------|-----------------------------------|------------------------------------|---------------------------|----------------------|------------------------------------------------------------------------------------------------------------------------------------------|
| 15791-1           | 1.5                               | 1,300                              | 90                        | 44                   | Sheet length, 65 in.                                                                                                                     |
| 15791-2           | 1.5                               | 1,100                              | 89                        | 97                   | Slight surface cracking noted on finished sheet. Sheet length, 72 in.                                                                    |
| 15791-3           | 1.5                               | 1,300                              | 90                        | 42                   | Sheet length, 75 in.                                                                                                                     |
| 15791-4           | 1.5                               | 1,300                              | 90                        | 42                   | Sheet length, 76 in.                                                                                                                     |
| 15791-4A          | 0.150                             | RT                                 | 10                        | 8                    | 15791-4 sheet was cut in 2 pieces. One piece 37 in. long was solution treated at 1600° F.-15 min. and WQ, followed by 10% cold reduction |
| 15791-4B          | 0.150                             | RT                                 | 10                        | 7                    | Second sheet, 39 in. long, from 15791-4 was solution treated at 1700° F.-15 min. and WQ, followed by a 10% cold reduction.               |
| 15791-2A          | 0.152                             | RT                                 | 10                        | 7                    | 15791-2 sheet was cut in 2 pieces solution treated at 1700° F.-15 min. and WQ, followed by a 10% cold reduction.                         |
| 15791-5           | 1.5                               | 1,100                              | 90                        | 87                   | Slight surface cracking noted on finished sheet. Sheet length, 83 in.                                                                    |

<sup>1</sup> The preheat temperature is that at which the material was allowed to soak. This soaking was performed in a 40 kw. resistance box furnace for 15 min. prior to each rolling pass. Whenever the material was allowed to air cool, it was preheated for a period of not less than 30 min. prior to the next rolling pass.

In the following tables of data summarizing the uniaxial tension test results for the alloys of this invention, the notation "R" indicates a practical measure of the texture achieved by any thermal-mechanical process. It measures the ratio of the plastic lateral strains, at 0.2% longitudinal plastic strains, measured in a uniaxial tension test performed on the alloy work piece regardless of the angular relation of the major axis of the work piece to the rolling direction. "R" is defined either as  $\epsilon_w/\epsilon_t$  or, alternatively, as  $d\epsilon_w/d\epsilon_t$  where  $\epsilon_w$  is the natural or logarithmic strain measured in the width dimension, and  $\epsilon_t$  is the similar measurement in the thickness dimension of the uniaxial tension test work piece. The same notation "R" is also used in the following discussion.

| 65  | Annealed at 1,400° F.-1 hr., ST 1,800° F.-1/4 hr. WQ, aged at 900° F.-24 hr. | Annealed 1,400° F.-1 hr., ST 1,800° F.-1/4 hr. WQ, aged at 900° F.-24 hr. |
|-----|------------------------------------------------------------------------------|---------------------------------------------------------------------------|
| 70. | Yield strength at 0.2% (k.s.i.) ----- 134.2                                  | 164.0                                                                     |
|     | Engineering tensile strength (k.s.i.) ----- 136.2                            | 184.0                                                                     |
|     | Young's modulus (p.s.i. $\times 10^{-6}$ ) ----- 15.6                        | 18.5                                                                      |
|     | Plastic strain at maximum load (percent) ----- >8                            | 2.2                                                                       |
|     | Total elongation (2-in. gage) (percent) ----- 20.8                           | 3.9                                                                       |
|     | Elastic Poisson's ratio ----- 0.443                                          | 0.349                                                                     |
|     | R at 0.2% long. plastic strain ----- 3.19                                    | 1.46                                                                      |
|     | Calculated 1:2 biaxial YS (k.s.i.) ----- 192.1                               | 202.5                                                                     |

75. NOTE.—Multi-directional rolled ~ 80%; furnace temperature 1,300° F.

TABLE VIII  
[Uniaxial tension data on Ti-7Al-2.5Mo alloy]

| Mechanical property                        | Conditions |       |       |
|--------------------------------------------|------------|-------|-------|
|                                            | A          | B     | C     |
| Yield strength at 0.2% (k.s.i.)            | 108.3      | 134.2 | 136.2 |
| Engineering tensile strength (k.s.i.)      | 121.8      | 156.5 | 157.2 |
| Young's modulus (p.s.i. $\times 10^{-6}$ ) | 16.2       | 16.4  | 16.0  |
| Plastic strain at maximum load (percent)   | ~4         | 4     | 2.5   |
| Total elongation (2-in. gage) (percent)    | 13.5       | 9.6   | 9.2   |
| Elastic Poisson's ratio, $\mu E$           | 0.368      | 0.420 | 0.382 |
| R at 0.2% longitudinal plastic strain      | 1.17       | 4.3   | 4.6   |
| Calculated 1:2 biaxial YS (k.s.i.)         | 128.5      | 203.0 | 208.1 |

Explanation of conditions: A—Hammer forged from 2-in. thick plate to 1-in. thick plate, furnace temp. 1,750° F. (as received). B—Material A, multidirectional rolled, furnace temp. 1,450° F. from 1 in. thick to  $\frac{3}{8}$  in. thick. Annealed at 1,400° F.-1 hr., ST at 1,750° F.- $\frac{1}{4}$  hr., WQ plus age at 900° F.-24 hr. C—Straight rolled from 1-in. thick plate to  $\frac{3}{8}$ -in. thick plate furnace temp. 1,750° F. Subsequently multi-directional rolled furnace temp. 1,400° F. from 0.621 in. to 0.125 in. Annealed at 1,400° F.-1 hr., ST at 1,750° F.- $\frac{1}{4}$  hr. WQ plus age at 900° F.-24 hr.

5

10

|                                            |       |
|--------------------------------------------|-------|
| Plastic strain at maximum load (percent)   | 5     |
| Total elongation (2-in. gage) (percent)    | 6.5   |
| Elastic Poisson's ratio                    | 0.359 |
| R at 0.2% long. plastic strain             | 1.98  |
| Calculated 1:2 biaxial YS (k.s.i.)         | 192.8 |
| Rolled 1500° F., annealed 1400° F., STA    |       |
| Mechanical property:                       |       |
| Yield strength at 0.2% (k.s.i.)            | 147.5 |
| Engineering tensile strength (k.s.i.)      | 165.6 |
| Young's modulus (p.s.i. $\times 10^{-6}$ ) | 15.6  |
| Plastic strain at maximum load (percent)   | 2.8   |
| Total elongation (2-in gage) (percent)     | 8.6   |
| Elastic Poisson's ratio                    | 0.356 |
| R at 0.2% long. plastic strain             | 1.75  |
| Calculated 1:2 biaxial YS (k.s.i.)         | 188.2 |

The uniaxial tension test work pieces were instrumented with strain gages to provide the test results. Initially, six

TABLE IX  
[Uniaxial tension data on Ti-6Al-4V, straight rolled, 90% reduction]

|                                            | As-rolled, 90% reduction <sup>1</sup> |               |                 | Annealed at 1,400° F.-1 hr. |                          |                 | Annealed at 1,400° F.-1 hr.<br>plus STA |               |                 | ST 1,700° F.- $\frac{1}{4}$ hr. WQ,<br>aged at 900° F.-24 hr. |               |                 |
|--------------------------------------------|---------------------------------------|---------------|-----------------|-----------------------------|--------------------------|-----------------|-----------------------------------------|---------------|-----------------|---------------------------------------------------------------|---------------|-----------------|
|                                            | Longitu-<br>dinal                     | Diag-<br>onal | Trans-<br>verse | Longitu-<br>dinal           | Diag-<br>Trans-<br>verse | Trans-<br>verse | Longitu-<br>dinal                       | Diag-<br>onal | Trans-<br>verse | Longitu-<br>dinal                                             | Diag-<br>onal | Trans-<br>verse |
| Yield strength at 0.2% (k.s.i.)            | 127.0                                 | 126.0         | 140.0           | 126.0                       | 124.0                    | 141.0           | 145.2                                   | 145.0         | 153.0           | 158.2                                                         | 146.0         | 150.6           |
| Engineering tensile strength (k.s.i.)      | 152.2                                 | 128.0         | 146.7           | 151.0                       | 127.5                    | 146.0           | 171.5                                   | 159.0         | 172.0           | 179.8                                                         | 162.0         | 172.0           |
| Young's modulus (p.s.i. $\times 10^{-6}$ ) | 14.9                                  | 18.3          | 17.3            | 15.15                       | 16.35                    | 19.0            | 15.75                                   | 16.8          | 15.75           | 15.9                                                          | 16.65         | 16.8            |
| Plastic strain at maximum load (percent)   | 5.8                                   | 5.7           | 2.2             | >8.0                        | >8.0                     | 5.0             | 3.6                                     | 4.0           | 2.4             | 4.8                                                           | ~3.0          | 5.0             |
| Total elongation (2 inches gage) (percent) | 9.0                                   | 17.8          | 4.5             | 18.1                        | 18.5                     | 14.2            | 10.4                                    | 11.0          | 8.7             | 7.1                                                           | 11.0          | 10.3            |
| Elastic Poisson's ratio                    | 0.350                                 | 0.378         | 0.395           | 0.341                       | 0.380                    | 0.406           | 0.353                                   | 0.391         | 0.391           | 0.317                                                         | 0.346         | 0.334           |
| R at 0.2% longitudinal plastic strain      | 1.33                                  | 4.08          | 0.9             | 1.17                        | 4.2                      | 0.83            | 1.66                                    | 3.32          | 1.76            | 0.85                                                          | 2.0           | 1.22            |
| Calculated 1:2 biaxial YS (k.s.i.)         | 154.0                                 | 188.2         | 158.8           | 149.7                       | 186.5                    | 158.0           | 183.5                                   | 208.5         | 195.2           | 177.6                                                         | 191.0         | 180.0           |

<sup>1</sup> From furnace temperature of 1,300° F.

In performing the several rolling schedules, the primary objective has been to achieve the highest possible lateral strain ratios through the development of a favorable crystallographic texture. Such a texture gives rise to high lateral strain ratios in uniaxial tension tests performed on work piece samples taken parallel to the rolling direction and transverse to the rolling direction. Thus, from the sheet materials that were rolled, emphasis was placed on measuring R in the rolling direction.

On the basis of a heat-treatment study and an indication that a 1400° F. anneal stabilizes the crystallographic texture, a standard heat treatment (STA) was adopted so that the influence of other processing parameters might be noted. This treatment consisted of a 1400° F.-1 hr. anneal, a 1700° F. solution treatment for  $\frac{1}{4}$  hr., water quenching, and aging at 900° F. for 24 hr.

strain gages were employed; two in the width dimension, on opposite faces; two in the thickness dimension on opposite edges; and two in the longitudinal dimension, on opposite faces. One-sixteenth-inch gage length, foil-type strain gages were used in the thickness direction and one-eighth-inch gage length foil-type strain gages were used in the length and width directions. All gages were bonded to the specimen surface with Eastman 910 contact adhesive.

A 2-in. gage length extensometer was also employed as a check of longitudinal strain. During each test, the load, the extensometer, and the six strain gages were read-out on eight channels of a light-beam oscilloscope. From the resulting data, lateral strain ratios were calculated at a number of points following the onset of plastic deformation.

From a comparison examination of the test results dis-

TABLE X  
[Uniaxial tension data on Ti-6Al-4V, multi-directional rolled 90%, furnace temperature 1,300° F.]

| Mechanical property                        | As-<br>rolled | Annealed<br>1,400° F.-<br>1 hr. | Annealed 1,400° F.-1<br>hr. ST 1,700° F.- $\frac{1}{4}$ hr., ST 1,700° F.- $\frac{1}{4}$ hr.<br>WQ, aged at 900° F.- $\frac{1}{4}$ hr. |               |                 | Annealed 1,400° F.-1<br>hr. ST 1,700° F.- $\frac{1}{4}$ hr., ST 1,700° F.- $\frac{1}{4}$ hr.<br>WQ, Aged at 900°<br>F.-24 hr. |
|--------------------------------------------|---------------|---------------------------------|----------------------------------------------------------------------------------------------------------------------------------------|---------------|-----------------|-------------------------------------------------------------------------------------------------------------------------------|
|                                            |               |                                 | Longitu-<br>dinal                                                                                                                      | Diag-<br>onal | Trans-<br>verse |                                                                                                                               |
| Yield strength at 0.2% (k.s.i.)            | 121.3         | 110.9                           | 146.0                                                                                                                                  | 143.0         | 148.3           |                                                                                                                               |
| Engineering tensile strength (k.s.i.)      | 130.8         | 114.5                           | 160.5                                                                                                                                  | 161.0         | 163.1           |                                                                                                                               |
| Young's modulus (p.s.i. $\times 10^{-6}$ ) | 14.25         | 15.0                            | 16.6                                                                                                                                   | 15.1          | 15.87           |                                                                                                                               |
| Plastic strain at maximum load (percent)   | 1.9           | 5.7                             | 4.5                                                                                                                                    | 3.0           | 3.2             |                                                                                                                               |
| Total elongation (2-in. gage) (percent)    | 11.1          | 15.3                            | 10.6                                                                                                                                   | 10.4          | 10.1            |                                                                                                                               |
| Elastic Poisson's ratio                    | 0.490         | 0.478                           | 0.495                                                                                                                                  | 0.403         | 0.399           |                                                                                                                               |
| R at 0.2% longitudinal plastic strain      | 3.35          | 4.72                            | 4.94                                                                                                                                   | 2.94          | 2.26            |                                                                                                                               |
| Calculated 1:2 biaxial YS (k.s.i.)         | 175.1         | 170.0                           | 225.5                                                                                                                                  | 201.4         | 198.7           |                                                                                                                               |

Note.—Uniaxial tension data on Ti-6Al-4V, multi-directional rolled 90%, furnace temperature 1,300° F.

closed in Tables IX and X, it can be seen that the multi-directional rolling process of this invention provides an alpha-beta type titanium alloy having a high strength to density ratio as indicated by the calculated R values. Table XI presents data resulting from a multi-directional rolling process conducted at temperatures of 1400° F. and 1500° F., respectively.

The invention has been described with particular reference to specific embodiments thereof. It is to be under-

TABLE XI

Uniaxial Tension Data on Ti-6Al-4V, Multi-Directional Rolled 90% Reduction at 1400° F. and 1500° F.

Rolled 1400° F., annealed 1400° F., STA

Mechanical property:

|                                            |       |
|--------------------------------------------|-------|
| Yield strength at 0.2% (k.s.i.)            | 147.5 |
| Engineering tensile strength (k.s.i.)      | 166.0 |
| Young's modulus (p.s.i. $\times 10^{-6}$ ) | 15.9  |

75

## 11

stood, however, that the description of the present invention is for the purpose of illustration only, and it is not intended to limit the invention in any way.

What is claimed is:

1. A method for rolling an alpha-beta titanium alloy sheet which comprises the steps of rolling said sheet to reduce its cross-sectional area by passing said sheet in a planar first direction parallel to the rolling direction in a single rolling pass while heated to a temperature between about 700° F. to 1500° F., continuing said rolling until the cross sectional area of the sheet is reduced by about 60 percent to 90 percent of its original cross-sectional area by performing a plurality of such rolling passes, angularly rotating said alloy sheet in the plane of said first direction subsequent to each repeated rolling pass such that rolling is effected in at least three differently oriented directions relative to said rolling direction and then cooling said rolled sheet to room temperature.

2. A method for rolling an alpha-beta titanium alloy sheet which comprises the steps of rolling said sheet to reduce its cross-sectional area by passing said sheet in a planar first direction parallel to the rolling direction in a single rolling pass while heated to a temperature of 1300° F., continuing said rolling until the cross-sectional area of the sheet is reduced to about 90 percent of its original cross-sectional area by performing a plurality of such rolling passes, rotating said alloy sheet 45° in the

## 12

plane of said first direction subsequent to each repeated rolling pass such that rolling is effected in at least three differently oriented directions relative to said rolling direction and then cooling said rolled sheet to room temperature.

5 3. A method in accordance with claim 2 wherein the rolled sheet is further annealed at a temperature of about 1400° F. for one hour, solution heat treated at 1700° F. for about 15 minutes, water quenched, and aged at 900° F. for 24 hours prior to cooling to room temperature.

10

## References Cited

## UNITED STATES PATENTS

|    |           |        |                                |
|----|-----------|--------|--------------------------------|
| 15 | 691,565   | 1/1902 | Norton.                        |
|    | 2,165,027 | 7/1939 | Bitter.                        |
|    | 3,169,085 | 2/1965 | Newman ----- 148—11.5          |
|    | 3,492,172 | 1/1970 | Sauvageot et al. ---- 148—11.5 |
|    | 3,496,755 | 2/1970 | Guernsey et al. ----- 72—364   |
| 20 | 3,489,617 | 1/1970 | Weurfel ----- 148—11.5         |

CHARLES W. LANHAM, Primary Examiner

E. M. COMBS, Assistant Examiner

## U.S. Cl. X.R.

25 148—12.7; 72—200, 364, 365, 700